

Patented Oct. 12, 1926.

1,602,590

# UNITED STATES PATENT OFFICE.

SAMUEL E. SHEPPARD, OF ROCHESTER, NEW YORK, ASSIGNOR TO EASTMAN KODAK COMPANY, OF ROCHESTER, NEW YORK, A CORPORATION OF NEW YORK.

## UTILIZATION OF BIOCHEMICAL LIGHT-SENSITIZING EXTRACTS IN THE ART OF PHOTOGRAPHIC MATERIALS.

No Drawing. Original application filed June 6, 1924, Serial No. 718,410. Divided and this application filed January 21, 1926. Serial No. 82,845.

This application is a division of my prior application 718,410 filed June 6, 1924 for art of light sensitive photographic materials, which has matured into Patent 1,574,-  
5 943, granted Mar. 2, 1926.

This invention relates to the art of photographic materials.

One object of the invention is to provide photographic sensitizing materials capable 10 of greatly increasing the light sensitiveness of photographic emulsions, especially of the developing-out type, even when incorporated therein in very small amounts. Another object is to provide such materials in 15 a concentrated and highly purified condition; so that they will not impair or harmfully dilute the emulsions in which they are used. A still further object is to provide processes for obtaining said materials 20 in said desirable condition.

Another object of the invention is to provide photographic emulsions, especially developing-out emulsions, having new and improved properties because of the use or 25 presence therein of my independent sensitizing materials. Still another object of my invention is to provide a process in which my said sensitizing materials are used to improve photographic emulsions, especially 30 developing-out emulsions, as regards light sensitiveness, by which term I include their ability to give the earliest visible impression or image with the minimum exposure or their ability to give density after a given 35 exposure or both, the usual photographic fluid treatments being used in preparing such impression or image.

A further object of the invention is to provide colloid products, such as treated 40 gelatin, the usefulness of which for forming light sensitive photographic emulsions, especially developing-out emulsions, is greatly increased and controlled by my said sensitizing material incorporated therewith. 45 Another object of the invention is to provide corresponding processes for making said intermediate colloid products.

Other objects are,—to increase the sensitiveness of photographic emulsions, particularly developing-out ones, while wholly or 50 partially dispensing with expensive or long and uncertain so-called ripening methods;

to enable the use of a type of gelatin having desirable physical qualities in making such a photographic emulsion of greater light 55 sensitiveness than that normally obtainable with said gelatin; to obtain more stable emulsions through the purity of the ingredients; to increase the light-sensitiveness of photographic emulsions, particularly 60 developing-out ones, the grain characteristics of which have already been determined; to increase the general light-sensitiveness of such photographic emulsions 65 throughout the spectral ranges to which they are normally sensitive; to make such photographic emulsions of standard light-sensitiveness characteristics with gelatins which normally do not produce emulsions having 70 such characteristics; to make, as intermediates in the manufacture of photographic emulsions, gelatins of standard light-sensitiveness giving power out of gelatins which do not normally have the power 75 of giving such standard sensitiveness to emulsions, such as developing-out ones, made from them. Further objects will hereinafter appear.

I have found photographic sensitizing materials, very small amounts of which 80 greatly increases the light-sensitiveness of photographic emulsions, such as those of the developing-out gelatino-silver-halid type for example. These materials I am able to prepare in especially concentrated and purified forms, so that when incorporated in 85 such emulsions or gelatins for such emulsions, they produce their sensitivity-increasing action without harmfully diluting said emulsions or gelatin or impairing the 90 physical properties and purity of them. Consequently my sensitizing materials supply safe, dependable, and practically independent means for controlling the properties 95 of photographic emulsions in addition to the customary expedients. The increases in sensitiveness of developing-out emulsions appear upon the usual developing, fixing, washing, and drying operations. Any customary developer, like the usual pyro or 100 metol-hydrochinon alkaline developers, are suitable for example.

The active sensitizing body or bodies in my sensitizing materials originate bio-

chemically in plants. It is found for instance in especially useful quantities in the sterol-containing extracts or fractions of plant extracts; although said compounds 5 may be even further purified and concentrated by whole or partial separation from the sterols. Fruitful and inexpensive sources of such active materials are by-products from cereal preparation, such as wheat, 10 bran, rice hulls, peas, and beans. Of course, cereal grains and leguminous plant seeds, are only mentioned as illustrative of the many vegetable organic tissues from which my sensitizing materials may be prepared.

15 Different sources vary in the extent to which they contain sensitizing material; but their suitability can readily be determined by a simple test. A small sample of the source in question can be extracted 20 by a method selected from the examples hereinafter given and the extract added to an emulsion such as one hereinafter described. If the sample sensitizing material causes a good increase in the light-sensitivity 25 of the emulsion, then the tested source can all be usefully extracted. This extraction of a sample and trial in a known emulsion provides a ready test for raw-material; but the preferred sources listed hereinabove 30 are in general reliable sources when a test is dispensed with. It is preferable to use sources which have not been submitted to excessive oxidizing action, which tends to 35 destroy the sensitizing power of the material.

In preparing my sensitizing material, I 40 free it from certain of its originally or normally associated impurities, especially the bulky ones, and those which might impair or dilute photographic emulsions. Generally speaking the preferred preparation of the material rids it of impurities insoluble in alcohol or those insoluble in light petroleum products such as ligroin. These are 45 typical of the many organic solvents of my sensitizing compound which may be employed. When some of the solvent is to enter emulsion, one is selected which is substantially free from injurious action on the 50 emulsion, alcohol being particularly good in this respect. My preferred preparation likewise frees the material from mineral compounds.

I find upon separating the principal impurities from my sensitizing compounds 55 that the resulting materials prove to be in most cases sterol-containing fractions. Such a useful sensitizing sterol extract is, for example, one substantially all soluble 60 in alcohol or ligroin. In general these fractions are substantially free from water-insoluble impurities as well as free from at least part of the water-soluble but alcohol-insoluble or ligroin-insoluble impurities. 65 The purified sensitizing compounds or bodies

in dry form and paste form and in the form of solutions are capable of increasing the sensitiveness of photographic emulsions, when incorporated therein and so the term sensitizing material applies to any one of 70 these forms.

While my invention is of wide utility in this art, it is especially useful in connection with gelatino-silver-halid emulsions such, for example, as developing-out emulsions employed on negative or positive films, 75 plates, papers, etc. The ammonia or alkaline type of such emulsions respond especially readily to my sensitizer. I shall, therefore, describe certain illustrative embodiments of my invention in connection with such emulsions; but it will be understood that my invention is not restricted to these examples but can be embodied in many 80 other species. 85

In the following examples there will be described the preparation of my sensitizing material from vegetable sources. Wheat 90 grains, corn, beans, peas, unhulled rice, wheat bran, mustard seeds, and rice hulls are a few illustrations of the types available. Mustard seeds are the most fruitful source. They are preferably comminuted and then extracted. For instance, lima beans are first ground to a coarse flour,—sufficiently fine to expose a large aggregate 95 surface to the extracting liquid. This flour, without being stored long enough to have its sensitizing material badly oxidized by the air, or volatilized, is extracted with ligroin boiling between 40° and 60° in a Soxhlet type of extractor until the operation is completed say for about 5 or 6 hours; although a longer time does no harm. For each kilogram (or 15,400 grains) of bean 100 flour it is convenient to use 3½ liters (or 56,600 mins.) of ligroin. The resulting extract is strong in sensitizing material and free from ligroin-insoluble material. It is 105 preferably evaporated to dryness and the residue taken up in alcohol, say 1 liter (or 17,000 mins.) for each 3½ liters (or 56,600 mins.) of the original ligroin extract. While the sensitizing material is thus finally 110 dissolved in alcohol, it is free from its ligroin-insoluble originally associated impurities, because ligroin was used in the 115 primary extraction. 120

Mustard seed, for another illustration, is ground in water, allowed to ferment for overnight, or say 12 hours, at room temperature. Then the mash is extracted, say by shaking with ligroin.

This solution is a strong sensitizing 125 material but can be concentrated and purified still further, if saponifiable oils be present in troublesome amounts. To remove such oils there is added to each liter of the final alcoholic extract, about 300 cc. (or 5,100 mins.) of the alcoholic extract from 7 grams 130

(or 108 grains) of sodium hydroxide. Of course, the strength of this saponifying alkaline solution can vary and equivalent solutions, like alcoholic potassium hydroxide be substituted. The mixture is boiled in apparatus having a reflux condenser, until the oils are saponified. The solution is then evaporated to dryness and the residue taken up in sufficient water for that purpose.

10 Ligroin or related petroleum ether is added with shaking. The sensitizing material enters the ligroin while the saponified oils and any liberated glycerine stay in the water. The ligroin extract is then separated out.

15 It is convenient to use 661 cc. (or 11,220 mins.) of ligroin in this extraction for each liter (or 17,000 mins.) of alcoholic extract subjected to the saponification treatment. The ligroin is next evaporated off

20 and the residue taken up in alcohol, 330 cc. (or 5,610 mins.) for each 660 cc. (or 11,220 mins.) of the ligroin from which the residue came. The finished alcoholic extract, which is likewise the sterol fraction from the beans,

25 is a very powerful sensitizing material, purified from fogging agents and from greasy or oily impurities. It is likewise substantially free from nitrogenous and mineral compounds.

30 The final alcoholic sterol extracts containing the sensitizing compounds, such as the extracts described above from vegetable sources are very useful but can be purified or concentrated even further by removing

35 the sterols, either wholly or partially. The sterols are substantially harmless to emulsions but are by themselves practically free from sensitizing actions, consequently their separation is useful. This can be done, for

40 example, by evaporating the sterol-containing fraction to dryness, taking up the dried residue in just enough warm but not boiling ethyl alcohol, say at 70° to 80° C., to dissolve it, cooling until sterol crystals form, removing said crystals, as by filtering, washing the crystals with a little ligroin, adding the wash liquid to the liquid from which the crystals came, and finally concentrating the combined liquids preferably under less than

45 atmospheric pressure, by evaporation. Or the combined liquids can be evaporated to dryness and the residue containing the sensitizing compounds dissolved in alcohol. If this first removal is insufficient the process can be repeated.

50 My concentrated and purified sensitizing material whether in the form of a solution, a solid or a paste is very powerful. Important and useful increases in light-sensitivity of emulsions even occur when the actual sensitizing compounds or bodies in the sensitizing material are of the order of a fifty-thousandth to a four hundred-thousandth of the weight of the emulsion in which they are incorporated. Of course,

the sensitizing bodies can be incorporated in still larger proportions but these minute amounts illustrate their power. Too much sensitizing tends to produce fog in some emulsions of the developing-out type. An 70 excess should, therefore, be avoided. Usually the solids in the added extract in its purified form are less than one ten-thousandth of the weight of the emulsion (non-aqueous ingredients).

75 My sensitizing material is concentrated and free from bulky and harmful impurities, with which it was originally or normally associated. In other words the active sensitizing bodies are in general more 80 concentrated and purer in my material than in the sources from which they are derived. This makes it especially useful without either diluting them to an undesirable extent or introducing fogging or other harmful 85 impurities. Stated in another way it increases their light-sensitivity without deteriorating their other qualities, such as setting ability, melting point, viscosity, and grain-characteristics. It enables me to establish a ratio of sensitizing material to 90 silver halid in the emulsions which is independent of the ratio of gelatin to silver halid.

95 The sensitizing bodies in my material appear to be not truly soluble in water but to form colloidal solutions therein. Its solutions in alcohol and ligroin are true ones. My sensitizing material has a very useful stability provided excessive exposure to oxidizing influences is not allowed. It is generally neither markedly acid or alkaline although it withstands dilute acid and alkalis and can be used when such are present in the emulsions. Since it is substantially without fogging action on emulsions when used in the proper amount for sensitizing them it yields emulsions of surprising stability when their sensitiveness is considered, fogging being long delayed. I classify the material 100 as biochemical or organic in distinction from inorganic materials such as ammonia and silver nitrate for example. The alcoholic solutions are, of course, protected from 105 harmful bacterial action, the alcohol being 110 a preservative.

115 My sensitizing material acts as a so-called "chemical" sensitizer instead of an "optical" sensitizer. In other words it increases the "general" sensitiveness of photographic emulsions in which it is incorporated,—that is to light of substantially the same wave lengths as those to which the emulsion would be sensitive without the incorporation of my material; instead of merely increasing the sensitiveness to some narrow group of wave lengths. Unlike dyes the sensitiveness is increased throughout the normal spectral range of the emulsion instead at only those spectral points 120 125 130

corresponding to the spectral absorption of the sensitizing material. My material is effective in increasing the general light-sensitivity of orthochromatic, panchromatic, X-ray, and all special emulsions, as well as the ordinary or non-color sensitized ones. It can be added with dyes or before or after them. It is nearly colorless itself. It is preferably added separately or independently of the sensitizing dye, generally but not necessarily before any dye. It is especially effective in emulsions having, at least, slight alkalinity.

My sensitizing material may be used in many ways. Broadly it may be incorporated in emulsions or in colloids for emulsions or both. It can also enter the emulsion mixed with other ingredients thereof whether organic or inorganic. It gives added light-sensitivity to various emulsions having different speeds and other distinctive characteristics. While it may be added at different stages of emulsion manufacture, nevertheless, it can be very conveniently mixed into the emulsion when the latter is otherwise complete ready for coating. Since its action is immediate when incorporated, the coating need be delayed only long enough to mix in the sensitizing material. With the grain characteristics such as size distribution etc. already determined, and the other physical and photographic properties of the emulsion already taken care of at this stage, I can practically independently increase its light-sensitivity without impairing said other properties by adding my concentrated purified sensitizing material.

As will be clear to those skilled in this art, the proportion of sensitizing material added to the emulsions will vary according to the concentration of the sensitizing material and according to the increase in light-sensitivity which is desired. The alcoholic extracts hereinabove described can be added, as a basis for trial, in the proportion of from 10 to 25 parts of extract to 1000 parts by volume of the emulsion. This is of the order of magnitude of 2 per cent. Of course, larger proportions can be used, provided harmful dilution is avoided; smaller amounts can be used for slight increases in sensitiveness and more concentrated extracts can be employed, or even the dried residues therefrom.

Where different batches of emulsion fall below a required manufacturing standard of light-sensitivity, although they may be otherwise satisfactory, their sensitiveness can readily be brought up to standard by mixing in my sensitizing material, the proportion varying with the increase necessary to produce a uniform product. Emulsions having almost no practical light-sensitivity but having enough other desirable

qualities can be made usefully light-sensitive by my material. Thus the latter is useful in connection with emulsions having good initial light-sensitivity and those having almost no initial sensitiveness. The increase in sensitiveness can be effected in one step by thoroughly stirring all of the sensitizing material into the emulsion at one time; or it may be incorporated part at a time in successive steps.

The following example illustrates how light-sensitive photographic emulsion may be prepared and improved by the aid of my sensitizing material. Of course, my invention is not restricted to this illustration but is applicable in the cases of the very large number of widely different emulsions in this art. The emulsion forming operations hereinafter described are along the lines of known practice, see for instance "Die photographic mit bromsilber gelatine" by J. M. Eder, published in Halle, Germany in 1903 by Wilhelm Knapp as Part III of Eder's "Ausfuhrliches Handbuch der Photographic."

The two following solutions are made up, the parts being by weight:

(A) 900 parts of silver nitrate in 9,200 parts of water.

(B) 690 parts of potassium bromide and 50 parts of potassium iodide in 6,100 parts of water along with 300 parts of gelatin.

In mixing B, the halid salts are first dissolved the water and the gelatin then added to the salt solution. Solution B is then warmed, say to 140° F. or 150° F. for example; and the silver nitrate solution A is gradually added to it with constant stirring. It is preferable to warm solution A before adding it to B, say to 150° F. or 160° F. for instance. When solution A has been thoroughly incorporated in solution B, there are then added 43 parts of strong ammonia previously dissolved in 900 parts of water. The emulsion formed by these operations is allowed to stand for a short time, say 15 minutes to a half hour for example. Then 1050 parts of gelatin are dissolved in it with thorough mixing. The emulsion is next cooled, such as by keeping in a cool space, until it sets to a firm jelly. The latter is broken up, as by shredding, for instance, and thoroughly washed to remove soluble salts, such as potassium nitrate and any excess potassium halids. The wash water is, of course, cool enough not to melt the pieces of emulsion jelly. The washed emulsion is next remelted to 100° F. and 1050 parts of water soaked gelatin are thoroughly mixed into it, the temperature then being raised, say between 120° F. and 150° F., for instance, for a short time, say a few minutes. It is then cooled and set. It is of the ammonia or alkaline type of emulsion.

My sensitizing material may be usefully

incorporated at any stage of the above described process of preparing the emulsion, even being premixed with solutions A or B or with ammonia or with the gelatin, at the 5 initial stages. It is very convenient to add it to the otherwise complete, melted, emulsion prior to coating on supports at the final stages in the process of preparing the emulsion. For example, the emulsion is 10 melted and there is thoroughly mixed into it 25 parts by volume of my sensitizing material (say one of the alcoholic extracts described above) for each 1000 parts by volume of emulsion. Since the actual sensitizing bodies are in the colloidized solids in such preparation and since such solids total as only a small proportion of said preparation (generally far less than one twenty-fifth) it follows that the actual sensitizing bodies are very useful when added in even less than one part per thousand of emulsion by weight. Often the ratio is less than one in ten-thousand or one in one-hundred-thousand. It will be noted that this 5 addition does not substantially dilute the emulsion, being of the order of two per cent.

With its light-sensitiveness increased by my material, the emulsion, being melted to the desired flowability, is coated on its support, such as glass, film, paper, etc., in the well known way. It is convenient to control and check the process by coating samples of the emulsion before and after the addition of my sensitizing material, the 5 coated specimens being tried out photographically by any well known sensitometric test, or even by comparative camera exposures on the same subject, under like conditions. Of course, the usual precautions are observed during the emulsion making and coating processes such as the use of non-actinic or "safe" light, cleanliness of vessels and air, etc.

The different gelatins sold for photographic emulsion-making may be used in the example given above, hard ones being very useful. The temperatures given, are, of course, adjusted if the particular gelatin employed has physical properties, such as melting and setting points, which deviate considerably from the usual ones, such adjustment being a matter of routine control.

Instead, however, of using gelatins which give emulsions of useful but lower sensitiveness even before the addition of my sensitizing material, an almost inert gelatin may be employed,—one which forms an emulsion which produces a developable image only after impractically long exposures, and then does not yield an image of desirable density. A gelatin which forms such a nearly inert emulsion may be prepared in the way described under the heading "Preparation of ash-free gelatin" in pages 1856 and 1859 of the "Journal of the

American Chemical Society," September, 1922, Vol. XLIV, No. 9, being part of an article by Sheppard, Sweet and Benedict on "Elasticity of purified gelatin jellies as a function of hydrogen-ion concentration." 70 Emulsions of impractically low light-sensitiveness made by the above described process from such prepared gelatin, are transformed by my sensitizing material into emulsions which give developable images of excellent density after usefully brief exposures. I have, for example, been able to increase the light-sensitiveness of such low sensitive emulsion over twenty times, the exposures for a given subject being cut to 80 less than one-twentieth of the original one and the image density being made excellent by a corresponding gain. Usually the percentage increase in light-sensitiveness is at least ten times the percentage increase in volume of the emulsion caused by the addition of material producing said increases. Often it is very much more indeed. Increases of the same general order of magnitude are made when my sensitizing material is added 85 in similar proportions to emulsions which are made from normal photographic gelatins or mixtures of such normal gelatins with said almost inert gelatins, and already have useful, but lower initial sensitiveness. 90 Different percentages of sensitizer produce correspondingly different increases. The increases in developing-out emulsions appear upon the usual developing, fixing, washing and drying operations. 95

For testing the power of sensitizing material, an almost inert emulsion made, as above described from said prepared gelatin is also very useful. Ten to twenty-five parts by volume of the sensitizing liquid 100 can be added to 1000 parts of such emulsion and the mixture coated and tested photographically in comparison with a parallel sample of the unsensitized emulsion. While the addition of sensitizing material as a 105 liquid is most convenient, the residue obtained from evaporating off the water from said liquid can be added directly to the emulsion. But a liquid spreading agent is preferable. In addition to having increased 110 sensitiveness, emulsions containing my sensitizing material have improved stability or keeping qualities because of the purification of said material. 115

My sensitizing material may be incorporated into gelatin with which photographic emulsions are to be made. This "strengthened" gelatin then constitutes a valuable intermediate in emulsion manufacture. For example, the gelatin can be melted and 120 to 25 parts by volume of my above described aqueous sensitizing material can be thoroughly mixed into 1000 parts of gelatin. Emulsions made from the mixture have increased light-sensitiveness as compared with 125 130

those made from corresponding unstrength-  
ened gelatin. The proportion of sensitizing  
material is, of course, adjusted to give  
the desired control of the sensitiveness of  
emulsions made from the gelatin, the total  
sensitizing material in the "strengthened"  
gelatin being thus brought above normal.  
It is especially effective when used in mak-  
ing emulsions having a slight alkalinity.  
10 In the examples given above the steps of  
treating with ammonia and warming of the  
emulsion just before its final setting im-  
prove the photographic properties of the  
emulsion, especially when the latter is made  
15 from hard gelatins. But one or both of  
them may be omitted. In other words, my  
sensitizing material acts by itself to increase  
the light-sensitiveness, whether ripening  
steps be employed or not, and so can wholly  
20 or partially replace them. The effect of  
either or both of such steps, however, is to  
help increase the light-sensitiveness of the  
emulsions and thus give a stronger initial  
sensitized condition which is multiplied  
25 or increased by using my sensitizing ma-  
terial. When using the ash-free gelatin  
mentioned above, they are especially readily  
dispensed with; but if retained in making  
very sensitive emulsions, they can be short-  
30 ened and made more certain in effect by  
reason of the use of my powerful and de-  
pendable sensitizing material. I consider  
the materials containing said compounds to  
be concentrated when they give a useful sen-  
35 sitizing effect without harmfully diluting  
the emulsions. My materials do not act as  
a photographic developer.

I have described gelatin emulsions because  
at the present time they are the ones which  
40 have the widest practical use. Moreover  
they form the best medium for testing my  
sensitizing materials, the characteristic ac-  
tion of such materials on such emulsions be-  
ing one of the best identifying criteria of  
45 such sensitizing materials. Other organic  
colloids and mixtures of them with each  
other or with gelatin, where their nature ad-  
mits such mixtures, may be used in making  
light-sensitive emulsions which can be im-  
50 proved by adding my sensitizing material.  
Albumens, agar-agar, gums, such as gum-  
arabic, cellulosic derivatives such as collodion  
are instanced. While I have disclosed the  
use of my sensitizer in connection with such  
55 sensitive substances as silver bromide and  
silver iodide, other light-sensitive substances  
can be employed, such as silver chlorid, alone  
or mixed with one or more of the others.

Having thus described my invention, what  
60 I claim as new and desire to secure by Let-  
ters Patent is:—

1. A photographic sensitizing material  
comprising a sterol-containing fraction of a  
biochemical extract dissolved in ligroin and  
having the property of increasing the gen-

eral light-sensitiveness of photographic gel-  
atino-silver-halid emulsions without increas-  
ing the grain-size thereof.

2. A photographic developing-out gela-  
tino-silver-halid emulsion of relatively high 70  
light-sensitiveness comprising a mixture of  
the constituents of a gelatino-silver-halid  
emulsion of lower light-sensitiveness and an  
independent sensitizing material upon which  
depends the difference between said lower 75  
and said high light-sensitiveness, said ma-  
terial comprising a sterol fraction of a bio-  
chemical extract substantially free from its  
ligroin-insoluble originally associated im-  
purities. 80

3. A photographic gelatino-silver-halid  
emulsion comprising gelatin, silver halid  
particles suspended therein, and an inde-  
pendent biochemical sensitizing extract, sub-  
stantially free from its originally associated 85  
ligroin-insoluble impurities, upon which ex-  
tract at least part of the light-sensitiveness  
of said emulsion depends, the physical prop-  
erties of said emulsion corresponding to the  
physical properties of said gelatin being sub-  
stantially unaltered by said sensitizing ex-  
tract. 90

4. In the process of making a photographic  
gela-  
tino-silver-halid emulsion, extracting 95  
a biochemical sensitizing material with lig-  
roin, and incorporating said extracted ma-  
terial in said emulsion to increase the light-  
sensitiveness thereof.

5. An intermediate for use in the making 100  
of photographic emulsions comprising an  
emulsion-forming colloid and an independent  
biochemical sensitizing material incorporat-  
ed therein, said material being substantially  
free from its normally-associated ligroin- 105  
insoluble impurities, said intermediate hav-  
ing the property of forming emulsions of  
higher general light-sensitiveness than those  
formed under parallel conditions from said  
colloid without said material.

6. A biochemical sensitizing material 110  
which has the property of increasing the  
light-sensitiveness of photographic gelatino-  
silver-halid emulsions when incorporated  
therein, said material being substantially  
free from its normally associated water- 115  
insoluble impurities and at least part of its  
normally associated water-soluble but  
ligroin-insoluble impurities.

7. In the process of preparing, from 120  
plant tissue containing the same, a sensitizing  
material having the property of increas-  
ing the general light-sensitiveness of photo-  
graphic gelatino-silver-halid emulsions  
when incorporated therein, the step of ex-  
tracting said tissue with a solvent of said  
material in which the bulk of said tissue  
is substantially insoluble, and incorporating  
sufficient of said material in such an emul-  
sion to increase the light-sensitiveness there-  
of. 125 130

8. In the process of preparing, from plant tissue containing the same, a sensitizing material having the property of increasing the general light-sensitiveness of photographic gelatino-silver-halid emulsions when incorporated therein, the steps of extracting said material from said tissue and concentrating said extract, and incorporating the concentrated extract in such emulsion to increase the general light-sensitiveness thereof. 45
9. In the process of preparing, from seedy tissues, a sensitizing material which has the property of increasing the general light-sensitiveness of photographic gelatino-silver-halid emulsions in which it is incorporated, the step of extracting said material from said tissues into an organic liquid which is a stronger solvent of said material than of the bulk of said tissues, and incorporating sufficient of said material in such an emulsion to increase the light-sensitiveness thereof. 50
10. In the process of preparing, from seedy tissues, a sensitizing material which has the property of increasing the general light-sensitiveness of photographic gelatino-silver-halid emulsions when incorporated therein, the step of extracting said material from said tissues with an organic solvent which is without substantially injurious action on said emulsions, and incorporating sufficient of said material in such an emulsion to increase the light-sensitiveness thereof. 55
11. In the process of making a photographic emulsion containing a biochemical colloid, extracting from active plant tissue a sensitizing material different from said colloid and incorporating sufficient of said material in said emulsion to increase the general light-sensitiveness thereof. 60
12. In the process of making a photographic gelatino-silver-halid emulsion, ex- 65
- tracting from active plant tissue by an organic solvent a sensitizing material and incorporating sufficient of said material in said emulsion to increase the light-sensitiveness thereof. 70
13. In the process of making a photographic emulsion containing a biochemical colloid, extracting a sensitizing sterol fraction independent of said colloid from a plant source and incorporating said fraction in said emulsion to increase the light-sensitiveness of the latter. 75
14. In the process of making a photographic emulsion containing a biochemical colloid, extracting from seedy tissue a sensitizing material and incorporating in said emulsion sufficient of said material to increase the light-sensitiveness thereof. 80
15. In the process of making a photographic biochemical colloid-sensitive-silver-salt emulsion, extracting a sensitizing material from seedy tissue in an organic solvent and incorporating said material in said emulsion. 85
16. In the process of making a photographic gelatino-silver-halid emulsion, extracting sensitizing material from seedy tissue, concentrating the extract, and incorporating it in said emulsion. 90
17. In the process of making a photographic gelatino-silver-halid emulsion, extracting a sensitizing material from seedy tissue in an organic solvent which is substantially without injurious action on said extract in said emulsion to increase the general light-sensitiveness thereof. 95
18. In the process of making a photographic emulsion containing a biochemical colloid, separating a sensitizing material from its associated seed tissue and incorporating it in said emulsion. 85

Signed at Rochester, New York this 18th day of January 1926.

SAMUEL E. SHEPPARD.